

Feb. 5, 1929.

1,700,973

C. F. BOOTH ET AL

NEUTRAL TRISODIUM PHOSPHATE

Filed July 19, 1924



Inventor

A. B. GERBER  
AND  
C. F. BOOTH

By

A. B. Gerber  
Attorney

## UNITED STATES PATENT OFFICE.

CHARLES F. BOOTH AND ARTHUR B. GERBER, OF ANNISTON, ALABAMA, ASSIGNEES  
TO FEDERAL PHOSPHORUS COMPANY, OF BIRMINGHAM, ALABAMA, A CORPORA-  
TION OF ALABAMA.

## NEUTRAL TRISODIUM PHOSPHATE.

Application filed July 19, 1924. Serial No. 726,918.

This invention relates to a new compound of sodium phosphate of a composition differing from that of ordinary tri-sodium phosphate, and preferably produced by the 5 method set forth in our co-pending application No. 726,917.

The tri-sodium phosphate found on the market at present contains more caustic soda than would appear necessary from the chemical formula generally said to represent that composition, viz:  $\text{Na}_3\text{PO}_4 \cdot 12\text{H}_2\text{O}$ . This statement is supported by several years' operation in producing ordinary tri-sodium phosphate as found on the market, and on examination of material produced by all manufacturers. As a result of this experience and these observations it is believed that the formula of commercial tri-sodium phosphate corresponds more nearly to



According to the equation



it would seem as if 10.5# NaOH would be sufficient to convert the di-sodium phosphate to tri-sodium phosphate on a basis of 100# of the latter; however, an average of several 30 years' operation is approximately 15# NaOH instead of the theoretical figure.

The presence of this additional quantity of caustic in ordinary tri-sodium phosphate may be determined by a titration of the 35 crystals. An examination of numerous samples from various manufacturers gave an average of 0.535 for a relation or "ratio" of the titration of the phenolphthalein to a titration of the same quantity of the methyl orange end point. This "ratio" is derived by dividing the cubic centimeters of standard acid used for the phenolphthalein titration, by the sum of the cubic centimeters of standard acid used for the methyl orange 40 titration. For example, if a given quantity of ordinary tri-sodium phosphate required 3.75 cc. half normal hydrochloric acid for the phenolphthalein titration and 3.25 cc. half normal hydrochloric acid for the methyl orange 45 titration the "ratio" would be 0.535. The formula for such a compound would cor-

respond to  $7(\text{Na}_3\text{PO}_4 \cdot 12\text{H}_2\text{O})\text{NaOH}$ . It was during the experiments conducted with a view to reducing the quantity of caustic soda required that it was found tri-sodium could 55 be produced with a formula  $\text{Na}_3\text{PO}_4 \cdot 12\text{P}_2\text{O}_7$ , as generally applied to tri-sodium phosphate. From the titration method as outlined above, it was apparent that the two compounds were of different composition and accordingly tri- 60 sodium phosphate, as now generally made, is an alkaline tri-sodium phosphate, while our new compound is a neutral tri-sodium phosphate.

In the production of this neutral tri-sodium phosphate the variations of specific gravity require corresponding variations of the "ratio" to produce neutral tri-sodium phosphate. In the chart the crystallization area curves A—B, C—D illustrate in area M how 65 if the specific gravity is too high with reference to the "ratio" some di-sodium phosphate will be formed, while in area O it is shown how if the "ratio" is too high with reference to the specific gravity some alkaline tri- 70 sodium phosphate will be formed. The area N indicates the conditions under which the neutral tri-sodium phosphate will form. 75

Area N lies between curves A B, along specific gravity ratios from 1.30, ratio 0.425 80 and 1.39 specific gravity, ratio 0.450; and curve C D, along specific gravity 1.308, ratio 0.395 and 1.39 specific gravity, ratio 0.445.

Having thus described our invention, what we claim as new and desire to secure by Letters Patent, is:—

1. The herein-described new composition of matter, consisting of a tri-sodium phosphate having no free alkali.

2. The herein-described new composition of matter, consisting of tri-sodium phosphate in crystalline form, in which the result of titration shows a ratio of 0.5 between the phenolphthalein end point and methyl orange 90 end point.

3. The herein-described new combination of matter, consisting of tri-sodium phosphate in crystalline form, containing no free alkali.

In testimony whereof we affix our signatures.

CHARLES F. BOOTH.  
ARTHUR B. GERBER.